

# UNITED STATES PATENT OFFICE.

ISIDOR POPPER, OF PHILLIPSBURG, NEW JERSEY.

## IMPROVEMENT IN INKS FOR WRITING.

Specification forming part of Letters Patent No. **132,102**, dated October 8, 1872.

*To all whom it may concern:*

Be it known that I, ISIDOR POPPER, of Phillipsburg, in the county of Warren and State of New Jersey, have invented a new and Improved Compound for Indelible Ink; and I do hereby declare the following to be a full, clear, and exact description thereof, which will enable those skilled in the art to make and use the same.

This compound relates to an ink or writing-fluid which, when applied on writing-paper, cannot be removed without destroying the texture of the paper or leaving a mark which bears witness that the writing has been tampered with. My compound consists of indigo, spirit of hartshorn, carbon, (by preference lamp-black,) gum arabic, glycerine, and water; and these ingredients are mixed together in about the following proportion: Indigo, four parts, by weight; spirits of hartshorn, thirty parts; lamp-black, or other equivalent carbon, ten parts; gum arabic, six parts; glycerine, thirty parts; water, fifty parts. After these ingredients have been thoroughly and intimate-

ly mixed, the ink or writing-fluid is put up in suitable bottles ready for the market.

My ink is intended particularly for the purpose of writing bank-checks, drafts, or other documents of value, since words, figures, or other signs or characters produced by my ink on writing-paper cannot be removed without producing marks showing that an attempt has been made to alter the check or other document.

I do not claim, separately, either of the ingredients herein named, for such, *per se*, is not new; but

What I claim as new, and desire to secure by Letters Patent, is—

A compound for writing-ink, consisting of lamp-black, glycerine, gum arabic, water, with or without hartshorn, made in the manner and in about the proportions specified.

This specification signed by me this 22d day of August, 1872.

Witnesses:

I. POPPER.

W. HAUFF,

E. F. KASTENHUBER.